

## UNITED STATES PATENT OFFICE

1,921,705

PROCESS FOR THE PRODUCTION OF  
ALUMINIUM SILICOSULPHIDE

Oskar Schober and August Schnitzspahn, Horrem, near Cologne-on-the-Rhine, Germany, assignors to American Lurgi Corporation, New York, N. Y., a Corporation of New York

No Drawing. Application June 30, 1932, Serial No. 620,306, and in Germany March 30, 1931

9 Claims. (Cl. 23—134)

This invention relates to a process for the production of aluminium silicosulphide.

The sulphides of aluminium and silicon, which could be usefully employed, for example, in vulcanizing rubber, are produced in known manner, by treating powdered aluminium or amorphous silicon with sulphur at elevated temperature. The preparation of pulverulent silicon, however, is expensive, as is also the reduction of aluminium to powder, in addition to which, in the latter case there is the known heavy risk of explosions in the pulverizing plant. Moreover, the reaction between aluminium and sulphur proceeds with such violence that losses of material 10 are hardly avoidable. For these reasons, therefore, none of the aforesaid sulphides has, so far, found practical application, notwithstanding their said suitability for vulcanizing rubber.

It has now been ascertained in accordance 20 with the present invention that the aforesaid inconveniences attending the production of the individual sulphides of aluminium and silicon can be obviated by producing their mixed sulphides jointly by treating with sulphur originating materials which contain both aluminium and silicon. This procedure affords, in the first place, the advantage that the originating materials may consist of aluminium-silicon alloys, which can be produced, for example by the thermal reduction of raw materials containing alumina and silica, at considerably lower cost than each of the components separately. Said originating alloys are available with particular advantage and at specially low prices, in the form 30 of liquation residues, comparatively high in silicon, obtained as a by-product in the conversion of the aluminium-silicon alloys—especially those high in silicon—obtained in the thermal reduction of aluminous and siliceous raw materials, into alloys that are lower in silicon, by liquation. The employment of such alloys affords the further advantage that these alloys are extremely brittle and can therefore be pulverized to any desired degree of fineness at low 40 cost and, above all, without risk of explosion. This is additionally facilitated by the fact that, when alloys obtained as by-products from liquation processes are employed, they already exist in a form which renders further pulverization 50 easy.

In general, such liquation products, containing for example about 35-40% of metallic Al and about 40-50% of metallic Si as they come from the liquation process, can be employed direct 55 for the production of the mixed sulphides ac-

cording to the present invention. Their composition may, however, be modified in any desired manner, by the addition of aluminium or silicon, or of an alloy higher in aluminium or silicon, prior to the action of the sulphur. 60

A further substantial advantage of the process of the present invention resides in the circumstance that the presence of the silicon moderates the energy of the reaction of the aluminium with the sulphur, the aforesaid unduly violent 65 reaction phenomena otherwise attending that reaction being prevented.

The components may also be employed, either wholly or in part, in the form of a mechanical admixture instead of in the form of an alloy. 70 In this case also, the advantage is obtained that the reaction with the sulphur can be performed in a single working operation, and that said reaction proceeds with less violence than that of pure aluminium with sulphur, the losses attending this latter reaction being consequently 75 prevented.

In carrying out the process of the present invention, the, for example, finely pulverized aluminium-silicon alloy, or finely powdered mixture of aluminium and silicon, is well mixed with sulphur—for example, in the form of flowers of sulphur—and the mixture is then brought into reaction by raising the temperature. Since the reaction is highly exothermic, it is usually sufficient to heat the reaction mixture—placed, for example, in a crucible or other reaction chamber bounded, for example, by refractory material such as chamotte—at only a single point. This may be effected by means, for example, of a red-hot iron rod, a primer of the kind used in alumino-thermic reactions, or in any other way. The reaction having thus been initiated in one portion of the mixture, it will then propagate 85 throughout the entire mass, by reason of the heat generated by the process itself. 90

It has been ascertained that special advantages are obtained by carrying out the said reaction in a molten state, i. e. by employing suitable working conditions, in order to ensure that the excess of the heat of the reaction per unit of time, plus any externally applied heat, over the heat losses, due to conduction and radiation, in the same period, is sufficient to bring the 100 mass into a state of fusion and maintain it in 105 that state throughout the reaction.

The following typical measures may be mentioned as suitable for the attainment of this object:

Employing the reaction components in a suffi- 110

ciently fine state of division. In general, it is advisable, for example, that the metallic components in particular—such as siliceous residues from the liquation of aluminium—silicon alloys—  
5 should be fine enough to pass through a sieve with not less than 3,600 meshes per sq. cm., for example one with about 10,000 meshes per sq. cm.

10 Avoiding any considerable—e. g. over 3%—excess of sulphur by comparison with the theoretical amount according to the equations:



15 It is preferable to employ the sulphur in amounts approximating to these equations. Nevertheless amounts which are both smaller and larger than the stoichiometric amounts of sulphur may be employed.

20 In operating without external application of heat and solely by initiating the conversion process by a brief heating of merely a portion of the reaction mixture to reaction temperature, it has also been found of advantage for rapidly  
25 fusing the reaction mixture, to employ for the ignition a fairly energetic agent, not merely a glowing iron rod or small primer, but a powerful igniting charge, in order to bring the mass into a state of fusion as quickly as possible. In place  
30 of or addition to the said means, any other convenient aids may of course be employed that are adapted, by the energetic initiation of the conversion process—and also, if desired, by the rapid application of considerable quantities of  
35 external heat—to accelerate the propagation of the reaction throughout the whole mass.

It has also been found desirable that the amounts of reaction mixture employed should not be too small, and that their spatial disposition should be such as to facilitate as far as possible the retention of the heat and the rapid propagation of the reaction; that is to say, preferably with a small surface of the mass in relation to its height.

40 It is important that the aforesaid ignition effected from above—for example, in a crucible filled with the reaction mixture—should take place as uniformly as possible over the entire cross-sectional area of the mass, under which conditions the reaction will proceed, in a stratified manner, from above downwards, over the whole cross section of the crucible.

45 For the purpose of reducing the heat losses, the crucible or other reaction apparatus may be provided with a heat-insulating shell.

50 Fresh quantities of the reaction mixture, in briquette form if desired, may be introduced into the wholly or partially molten mass, in the same manner, for example, as practised in the so-called aluminothermic process or the like.

55 When the conversion is completed, the resulting molten product may, if desired, be poured into moulds.

60 The molten products obtained in accordance with the present invention are distinguished, in comparison with those obtained when the reaction mixture is not fused during the conversion process, by their considerably higher content of

65 sulphide-sulphur decomposable by water with liberation of sulphuretted hydrogen. Products obtained from liquation residues for example with about 45 to 50% of metallic Si and 35 to 40% of metallic Al, treated according to the  
70 present invention, furnish, for example 45-50%

(or more) of their weight of sulphuretted hydrogen.

The mixed sulphides, especially those produced in the molten state, prepared in accordance with the process of the present invention, 80 have been found admirably suitable for a great variety of purposes, such as for example vulcanizing rubber, destroying pests, removing hair from the skins of animals, cosmetic purposes, the preparation of luminous paints, and for furnishing H<sub>2</sub>S for precipitating sulphides for manufacturing and analytical purposes and the like.

85 According to the purpose in view, the products obtained in the first place, in the form of a pulverulent, sintered or fused mass, may be reduced to a sufficiently fine condition, for example in enclosed ball mills, prior to being used.

90 For the purpose of preparing mixed sulphides containing additional sulphides, the alloy or mixture of aluminium and silicon employed as the originating material may, prior to the reaction with sulphur and, if desired, during the process of pulverization, be mixed with other metals or with metallic compounds, preferably 95 finely powdered, furnishing sulphides on treatment with sulphur under the reaction conditions. The aluminium-silicon alloy employed may also, in itself, already contain other metals 100 or other constituents in addition to the said 95 components.

95 An advantage which is of particular importance in connection with many applications of these products is that practically their entire sulphur content can be converted into sulphuretted hydrogen by mere treatment with water 110 without the aid of acids.

#### Example 1

115 20 kgs. of liquation residues (containing 35.5% of metallic Al and 44.5% of metallic Si) which had been obtained by liquating an Al-Si alloy for the purpose of recovering an alloy higher in Al, are pulverized to a degree of fineness corresponding to a sieve with 10,000 meshes per 120 sq. cm., and mixed with 36 kgs. of sulphur in powder form. This mixture is spread out in a shallow fireclay crucible and is touched at one spot with an iron rod at bright red heat. In 125 consequence of the resulting initiation of the conversion process, the whole mixture burns away, without, however, fusing. The scaly mass of aluminium silico-sulphide obtained when the reaction has terminated contains up to 8% 130 or more by weight of sulphur, and can be ground—for example in a ball mill—when cold.

#### Example 2

135 A mixture of 20 kgs. of the liquation residues employed in Example 1 (and of the same degree of fineness) with 32 kgs. of powdered sulphur is placed in a stout fireclay crucible, insulated to prevent loss of heat, 70 cm. deep and 38 cm. 140 wide inside. A priming charge of 500 grms. of a mixture composed of 178 grms. of powdered Al and 322 grms. of powdered Si is spread over the said mixture.

145 After igniting the priming charge with a match the conversion of the reaction mixture takes place within about 20 minutes, the whole mass passing into a state of fusion.

150 Directly the conversion is completed, the still fluid melt is poured into suitable moulds. The

resulting product contains 45-52% by weight of sulphur.

The term "mixed sulphides" used in the foregoing description is intended to include in all cases products consisting essentially of aluminum and silicon in chemical combination with sulphur, which products may additionally contain minor quantities of various substances such as iron, titanium, calcium, aluminum oxide, silicon carbide, silicic acid, and the like.

We claim:—

1. A process for the production of products consisting essentially of the sulphides of aluminum and silicon which comprises causing metallic aluminium, together with metallic silicon, to react with sulphur at elevated temperature.

2. A process for the production of products consisting essentially of the sulphides of aluminum and silicon which comprises causing metallic aluminium, in a finely divided state, together with metallic silicon, to react with sulphur by heating the reaction mixture to reaction temperature at one point at least.

3. A process for the production of products consisting essentially of the sulphides of aluminum and silicon which comprises causing metallic aluminium, in a finely divided state, together with metallic silicon, to react with sulphur by heating the reaction mixture to reaction temperature at one point at least, by burning an igniting charge.

4. A process for the production of products consisting essentially of the sulphides of aluminum and silicon which comprises causing a mixture of an alloy of aluminium with silicon in a

finely pulverized form, to react with sulphur at elevated temperature.

5. A process for the production of products consisting essentially of the sulphides of aluminum and silicon which comprises causing a mixture of metallic aluminium, metallic silicon and sulphur to react at elevated temperature.

6. A process for the production of products consisting essentially of the sulphides of aluminum and silicon which comprises causing metallic aluminium, together with metallic silicon, to react with sulphur, in a molten state.

7. A process for the production of products consisting essentially of the sulphides of aluminum and silicon which comprises causing a mixture of a finely powdered aluminum-silicon alloy, obtained by liquating an aluminum-silicon alloy containing a lower silicon content than that of the liquation product, to react with sulphur in a molten state.

8. A process for the production of products consisting essentially of the sulphides of aluminum and silicon which comprises causing a mixture of sulphur and a finely powdered aluminum-silicon alloy, obtained by liquating an aluminum-silicon alloy containing a lower silicon content than that of the liquation product, to react in a molten state by heating said mixture at one point by means of an energetic ignition charge.

9. As an article of commerce, a product consisting essentially of sulphides of aluminum and silicon.

OSKAR SCHOBER.  
AUGUST SCHNITZSPAHN. 110

40

115

45

120

50

125

55

130

60

135

65

140

70

145

75

150

80

85

90

95

100

105

110

115

120

125

130

135

140

145

150